

## UNITED STATES PATENT OFFICE

2,085,543

## PROCESS FOR COATING METALS

Floyd Francis Oplinger, Niagara Falls, N. Y., assignor to E. I. du Pont de Nemours & Company, Wilmington, Del., a corporation of Delaware

No Drawing. Application May 21, 1935,  
Serial No. 22,651

13 Claims. (Cl. 204--17)

This invention relates to the production of rust-proof coatings on iron and steel and other metals and has for an object an improved method for applying tin and tin alloy coatings to metallic articles, especially to iron and steel. A further object of the invention is to provide a means for transforming a relatively dull, electroplated tin or tin alloy coating to a bright, smooth, mirror-like coating. A further object is to produce bright, smooth coatings of electroplated tin on cold-rolled steel. Other objects will be apparent from the following description.

In my copending application Ser. No. 709,171, I have described and claimed a method for producing bright tin coatings on iron, steel and other metals, which method comprises first electroplating with tin, thereafter heat-treating the electroplated surface under substantially non-oxidizing conditions to fuse the tin electrodeposit and then cooling. This method, which is applicable to tin, fusible tin alloys and other fusible metallic electrodeposits, transforms the relatively dull electroplated coatings to bright, smooth, mirror-like surfaces which are highly corrosion resistant because the heat-treating operation effectively closes any pin holes, pores or crevices which may occur in the electrodeposit. In the said copending application I have disclosed that this method when applied to cold-rolled sheet steel does not produce the desired smooth appearance of the finished heat-treated article unless the steel is specially treated prior to electroplating by a method disclosed and claimed in said application. This method of pre-treating cold-rolled steel to cause the finished product to be smooth and bright rather than rough and lumpy consists in first treating the steel surface with an acid to such extent that the surface is distinctly and visibly etched and following this treatment with an alkaline treatment, e. g. anodic treatment in an alkaline bath, preferably one containing an alkali metal cyanide.

I have now discovered that by the employment of the herein described invention I may produce smooth, bright coatings of tin or tin alloy on cold-rolled steel and the like by first electroplating with the tin or tin alloy followed by heat treatment to the melting point of the electrodeposit under substantially non-oxidizing conditions, without applying the aforesaid acid etching-alkali treatment to the steel. I have found that this advantageous result may be accomplished by adding a small amount of a soluble compound of one or more of the following metals

to the tin or tin alloy electroplating bath: copper, nickel, silver or a cobalt, thereby simultaneously plating out a small amount of the metal whose compound has been added to the bath together with the tin or tin alloy electrodeposit. In arriving at this discovery, I have tested a number of various metals for this purpose and have found that only the metals enumerated above are suitable for accomplishing the desired result. For example, metals such as lead, cadmium, zinc and mercury are not suitable for use in the present invention. The presence of such metals does no harm as a rule, but in order to obtain smooth, bright coatings of tin or tin alloy by heat-treating the electrodeposit on cold-rolled steel, I have found it essential that at least one of the metals: copper, nickel, silver or cobalt be present in a small amount in the electrodeposit. By this means I have produced smooth, bright mirror-like coatings of tin upon various types of cold-rolled sheet steel without using the above described acid etch-alkaline pre-treatment prior to electroplating steel, the steel prior to electroplating being merely cleaned by any known process for removing grease, dirt and the like prior to electroplating. If desired, in practicing my invention the acid etch-alkaline pre-treatment may be used but this is not essential and ordinarily is not especially advantageous when practicing the herein described invention.

In one method of practicing the herein described invention, I may add to an ordinary tin electroplating bath a compound of copper, nickel, cobalt or silver soluble in the bath and electroplate the article to be coated in the bath, whereby an electrodeposit is obtained which contains a relatively small amount of the metal whose compound is added to the bath. Prior to electroplating, the article to be electroplated may be cleaned by any desired method to remove grease, dirt, oxide and the like. If an acid is used to remove oxide or scale, it is not necessary to continue the acid treatment to the point where visible etching occurs. When the desired thickness of electrodeposit has been obtained, the electroplated article is rinsed, dried, and then heated under substantially non-oxidizing conditions to a temperature slightly above the melting point of electrodeposit. The various methods of heat-treating under non-oxidizing conditions which are described in my aforesaid copending application are suitable for this step. For example, the plated article may be immersed in hot oil or molten tallow, heated in an atmosphere of substantially non-oxidizing gas such as

5

10

15

20

25

30

35

40

45

50

55

hydrogen, nitrogen, carbon vapor, or immersed in a molten salt bath. If desired, in these methods, electrical induction or electrical conduction may be used to heat the electroplated metal.

5 Preferably, the heat-treating is not prolonged much beyond the time required to obtain complete fusion of the electrodeposit and then is preferably cooled under conditions least favorable to oxidation, e. g. by quenching in cold water or

10 cold oil.

In practicing my invention, I prefer to use copper or nickel or both of these metals since these metals are less expensive than silver and cobalt and generally are more satisfactory for my purpose. By experimentation I have found that it is necessary to plate out relatively small amounts of copper or nickel on the cathode in order to produce the desired smooth, bright, mirror-like coats on subsequent heat-treatment.

15 20 For example, in order to produce the desired result, the tin electrodeposit should contain not less than about 1.4% of copper, or silver or not less than about 0.4% of nickel or cobalt. If the electrodeposit contains substantially less than 25 these amounts, the desired result usually is not obtained and on subsequent heat-treating the coating tends to be rough or lumpy and does not appear to adhere well to the underlying surface. It is to be understood that said lower limits of

30 35 copper or nickel suitable for practicing my invention are based on the specific methods of analysis which are described hereinafter in the examples given to illustrate my invention, which methods comprise an electrolytic method for determining copper and the use of dimethyl glyoxime for the determination of nickel. While generally satisfactory results may be obtained by plating out copper or nickel in the tin electrodeposit at or near to the lower limits above specified, I usually prefer to use some higher amounts of such metals to insure consistent results in extended periods of operation. Thus I prefer to operate so that the copper content of the electrodeposit is not less than about 2% by weight or, if nickel is used

40 45 instead of copper, so that the nickel content in the electrodeposit is not less than about 0.5% by weight. The melting point of the resulting electrodeposit obviously will depend upon the amount of copper or nickel content, the effect of large proportions of these metals being to raise the melting point of the electrodeposit. I prefer to adjust the copper or nickel content of the bath so that the melting point of the resulting composite electrodeposit is not greater than about

50 55 60 65 260° C. at or below which temperature the heat-treating operation may be conveniently carried out in a molten tallow bath. I have found that in order to obtain this result, the copper content of the electrodeposit should not exceed about 15% or the nickel content, if nickel is used, should not exceed about 2% by weight. By operating in this range, I have found that it is possible to obtain the desired results by heat-treating the electrodeposit under non-oxidizing conditions in a temperature range of about 230°-260° C.

My invention is further illustrated by the following examples:

#### Example 1

70 A plating solution was prepared, containing:

|                        | Oz. per gal. |
|------------------------|--------------|
| Sodium stannate-----   | 20           |
| Sodium hydroxide-----  | 1.5          |
| 75 Sodium acetate----- | 2            |

The solution was filtered and allowed to settle until thoroughly clear and then a quantity of  $\text{Ni}(\text{CN})_2 \cdot 2\text{NaCN}$  solution equivalent to 0.01 gm. per liter of nickel was added.

The bath was operated at 65° C., with Straits 5 tin anodes and cold-rolled sheet steel cathode at 15 amperes per square foot cathode current density. The bath was operated under these conditions twice daily on four consecutive working days for 1-hour periods as shown in the table 10 below. During each entire electroplating period, weighed cathodes of pure tin foil were plated in the bath and 2 to 3 cold-rolled sheet steel cathodes were simultaneously plated for 10 minutes each. The plated tin foil cathodes were analyzed 15 for nickel by the following procedure: The electroplated foil is washed, dried and weighed to determine the weight of the electrodeposit. The foil then is dissolved in a solution of 10 parts of concentrated nitric acid, 10 parts of concentrated hydrochloric acid and 25 parts of water. About 25 grams of sodium tartrate is added to the resulting solution to prevent precipitation of tin and the solution is made slightly alkaline with ammonium hydroxide. Nickel then is precipitated with dimethyl glyoxime and the precipitate 20 filtered off, washed, dried and weighed in the usual manner for the determination of nickel. Preferably, the precipitate is redissolved in hydrochloric acid, sodium tartrate added and the 25 nickel re-precipitated as described above. The 30 analytical results are shown in the following table:

| Day           | Time                                                      | Analysis of deposit                | 35 |
|---------------|-----------------------------------------------------------|------------------------------------|----|
| Thursday----- | 11:11-11:30 A. M.<br>12:10-3:10 P. M.<br>3:45-10:45 A. M. | 1.34% Ni<br>0.573% Ni<br>0.848% Ni |    |
| Friday-----   | 2:00-3:00 P. M.<br>10:00-11:00 A. M.                      | 0.718% Ni<br>0.427% Ni             | 40 |
| Monday-----   | 1:30-2:30 P. M.<br>9:50-10:50 A. M.                       | 0.382% Ni<br>0.452% Ni             |    |
| Tuesday-----  | 12:00-1:00 P. M.                                          | 0.481% Ni                          |    |

The electroplated steel cathodes were washed, dried and then heat-treated by immersing them 45 for 10 to 30 seconds in molten tallow maintained at a temperature of about 250° C. and cooled in the air. In each trial, the resulting heat-treated plate was smooth, bright and mirror-like.

#### Example 2

A tin plating solution was made containing the following ingredients:

|                       | Gms./L. |
|-----------------------|---------|
| Sodium stannate-----  | 150     |
| Sodium acetate-----   | 15      |
| Sodium hydroxide----- | 11      |

This bath was operated at a bath temperature of 70° C. in a cathode current density of 15 60 amps./sq. ft., using Straits tin anodes to electroplate samples of cold-rolled sheet steel. In order to simultaneously plate out copper with the tin from this bath, cuprous cyanide was dissolved in sodium cyanide solution and small amounts of this copper solution were added to the bath from time to time. After each addition of the copper cyanide solution to the bath, samples of cold-rolled steel were electroplated in the bath under the above mentioned conditions for 15 minutes 70 and at the same time a weighed sheet of pure tin foil was also electroplated for the same period of time. The sheet steel cathodes, after electroplating, were washed, dried and then heat-treated at 230°-260° C. by immersing in a heated bath of 75

molten tallow. The electroplated tin foil was analyzed for copper content by the following method: The plated foil was washed, dried and weighed and then was dissolved with a large excess of 50% nitric acid solution and the solution evaporated down to a dry powder at a temperature of 100° C. The resulting powder was treated with 25 cc. of concentrated nitric acid and 75 cc. of water and heated to approximately 80° C. and the hot solution was filtered through No. 1 filter paper. The precipitate on the filter was thoroughly washed with 1% nitric acid to remove all traces of copper and the washings combined with the filtrate. The resulting clear solution was electrolyzed, using platinum gauzes as anode and cathode with 2 amperes of current. Electrolysis was continued until there was no further gain in weight of the cathode. The cathode then was dried and weighed to determine the amount of copper in the tin electrodeposit. The results obtained are shown in the following table:

| 25 | Sample | CuCN added to plating bath | Copper in electrodeposit | Appearance of electrodeposit on steel cathode after heat treatment |
|----|--------|----------------------------|--------------------------|--------------------------------------------------------------------|
|    |        |                            |                          |                                                                    |
| 30 | 2----- | 0.01                       | Trace                    | Very rough—poor adherence to steel.                                |
| 30 | 3----- | 0.05                       | 0.21                     | Better than Sample 1, but lumpy.                                   |
| 30 | 3----- | 0.10                       | 1.39                     | Good adherence—slight tendency towards lumpiness.                  |

### Example 3

A tin plated bath was prepared having the following composition:

|    |                       | Oz./gal. |
|----|-----------------------|----------|
| 40 | Sodium stannate-----  | 20       |
|    | Sodium acetate-----   | 2        |
|    | Sodium hydroxide----- | 1.5      |

Various amounts of a sodium-copper cyanide solution of known copper concentration were added to the bath from time to time and after each addition cold-rolled sheet steel cathodes were electroplated in the bath, using Straits tin anodes and a cathode current density of 15 amperes per square foot. At the same time sheets of tin foil were electroplated with the same cathode current density. The electroplated steel cathodes were heat-treated as described in Example 3 while the plated tin foil samples were analyzed for their copper content, whereby the copper content in the electrodeposit was determined. All of the electrodeposits (except that of Sample 8 which contained 23.6%) were transformed to smooth, bright, mirror-like coatings by the heat-treatment. In the case of Sample 8, the melting point of the electrodeposit, because of the high copper content, was above 260° C. and therefore the heat treatment failed to fuse the coating. The results obtained are shown in the following table:

| 65 | Sample | Cu content of deposit | CuCN content of bath |
|----|--------|-----------------------|----------------------|
|    |        |                       |                      |
| 70 | 1----- | 1.07                  | 0.12                 |
|    | 2----- | 9.0                   | 0.57                 |
|    | 3----- | 10.0                  | 0.49                 |
|    | 4----- | 14.6                  | 0.97                 |
|    | 5----- | 9.0                   | 1.46                 |
|    | 6----- | 12.01                 | 1.10                 |
|    | 7----- | 10.9                  | 1.43                 |
|    | 8----- | 23.6                  | 3.54                 |

### Example 4

Cold-rolled sheet steel was electroplated at 15 amperes per square foot cathode current density, from a tin plating bath having the composition of the bath of Example 1, except that 2 gms. per liter of a silver cyanide (dissolved in sodium cyanide solution) was added in place of nickel cyanide. The electroplated steel, on heating in molten tallow at 245° C. readily fused, forming a smooth coating. 10

### Example 5

Cold-rolled steel was electroplated as in Example 4, except that in place of silver cyanide, sodium cobaltcyanide was added to the bath in an amount equivalent to 4.5 gms. per liter of cobalt. On heat-treating in molten tallow, a bright, smooth tin coating was obtained. The tin electrodeposit was found by an analytical method similar to that of Example 1 to contain 0.35% of cobalt. Similar trials, using smaller amounts of cobalt, produced rough, lumpy deposits on heat-treating at 245° C. 15 20

In practicing my herein described invention, I prefer to add to the electrolyte an amount of soluble compound of copper, nickel, silver and/or cobalt not less than about 0.01 gram per liter, in order to insure that there always will be sufficient of the added metal in the bath to plate out the desired amount of such metal in the electrodeposit. In the operation of tin or tin alloy plating baths, a precipitate of tin oxide sometimes forms which slowly settles to the bottom of the electroplating tank. During operation, the electrolyte often becomes more or less stirred up, e. g. by the passage of work therethrough and I have found that if the bath containing tin oxide or other tin precipitate is stirred up and then allowed to settle, there is a tendency for the settling material to adsorb or occlude some of the added copper or nickel compound and thus decrease its concentration. To avoid concentration of the added metal compound being thus unduly decreased, I prefer to maintain its concentration in the bath not lower than 0.01 gram per liter and preferably 0.05 to 1.5 grams per liter or higher. For example, when operating by the addition of sodium-copper cyanide to an alkaline tin plating bath, I prefer to maintain the copper cyanide concentration in the bath at from 0.05 to 1.5 grams per liter and if operating by the addition of dissolved nickel cyanide I prefer to maintain the nickel cyanide concentration at between 0.1 to 0.4 gram per liter. In ordinary plating operations, the required concentration of the added metal to the electroplating bath may readily be maintained by periodical additions of the metal compound at periodic intervals, e. g. once or twice daily. When starting the operation of a freshly made tin electroplating bath in accordance with my invention, I prefer to allow the electrolyte to settle or to filter it before the salt of copper, nickel, etc. is added thereto. 35 40 45 50 55 60 65

My herein described invention is not restricted to the above described specific methods of operation which have been set forth by way of example. For example, instead of adding copper, nickel, cobalt and/or silver compound to the tin plating bath in order to obtain an electrodeposit containing such metal, I may electroplate alternate layers of tin and the added metal from separate plating baths. Thus I may electroplate a thin layer of copper or nickel on an electrodeposited tin layer and subject the resulting electrodeposit 70 75

to the heat-treating operation, with satisfactory results. It is preferable, however, to simultaneously plate the tin and added metal from a single electrolyte, since this generally results in better 5 distribution of the added metal throughout the coating layer.

My invention, while particularly adapted for coating cold-rolled sheet steel and similar cold-worked ferrous metal articles, is equally useful for 10 plating other ferrous metal articles, e. g. hot-rolled steel sheet, steel wire and the like and non-ferrous metals having sufficiently high melting points to withstand the required heat-treatment, 15 e. g. copper, brass, bronze and the like. My method results in smooth, mirror-like coatings of high corrosion resistance on the various metals to which it may be applied. The only preparatory treatment required prior to the electroplating 20 step is the usual treatment for removing oxide, grease and dirt which is ordinarily used in electroplating operations.

I claim:

1. A process for coating a cold rolled steel surface, comprising electroplating said surface with 25 a tin alloy consisting preponderantly of tin and containing at least one metal selected from the group consisting of copper, nickel, silver and cobalt and thereafter heating the electroplated surface under substantially non-oxidizing conditions 30 to a temperature above the melting point of the electrodeposit and then cooling.

2. A process for coating cold-rolled steel comprising electroplating said steel from a tin bath containing not less than about 0.01 gram per liter 35 of a dissolved copper compound and thereafter heating the electroplated steel under substantially non-oxidizing conditions to a temperature above the melting point of the electrodeposit and then cooling.

40 3. A process for coating cold-rolled steel comprising electroplating said steel from a tin bath containing not less than about 0.01 gram per liter of a dissolved nickel compound and thereafter heating the electroplated steel under substantially non-oxidizing conditions to a temperature 45 above the melting point of the electrodeposit and then cooling.

4. A process for coating cold-rolled steel comprising electroplating said steel from an alkaline 50 tin plating bath containing about 0.05 to 1.5 grams per liter of dissolved cuprous cyanide and thereafter heating the electroplated steel under substantially non-oxidizing conditions to a temperature above the melting point of the electrodeposit and then cooling.

5. A process for coating cold-rolled steel comprising electroplating said steel from an alkaline tin bath containing about 0.1 to 0.4 grams per liter of dissolved nickel cyanide and thereafter heating the electroplated steel under substantially non-oxidizing conditions to a temperature above the melting point of the electrodeposit and then cooling.

6. A process for producing a bright, smooth 65 coating of tin on cold-rolled steel comprising simultaneously electroplating the surface of said steel with tin and another metal selected from the group consisting of copper, nickel, silver and

cobalt in such manner that the resulting electrodeposit consists preponderantly of tin and contains an amount of said other metal not less than about 0.4% by weight when said other metal is nickel or cobalt and not less than about 1.4% 5 when said other metal is copper or silver and thereafter heating the electroplated steel under substantially non-oxidizing conditions to a temperature above the melting point of said electrodeposit.

7. A process for producing a bright, smooth coating of tin on cold-rolled steel comprising simultaneously electroplating said steel with tin and copper in such manner that the resulting electrodeposit consists preponderantly of tin and contains not less than about 1.4% by weight of copper and thereafter heating the electroplated steel under substantially non-oxidizing conditions to a temperature above the melting point of said electrodeposit.

8. A process for producing a bright, smooth coating of tin on cold-rolled steel comprising simultaneously electroplating said steel with tin and copper in such manner that the resulting electrodeposit consists preponderantly of tin and contains about 2 to 15% by weight of copper and thereafter heating the electroplated steel under substantially non-oxidizing conditions to a temperature of about 230° to 260° C.

9. A process for producing a bright, smooth 30 coating of tin on cold-rolled steel comprising simultaneously electroplating said steel with tin and nickel in such manner that the resulting electrodeposit consists preponderantly of tin and contains not less than about 0.4% by weight of nickel 35 and thereafter heating the electroplated steel under substantially non-oxidizing conditions to a temperature above the melting point of said electrodeposit.

10. A process for producing a bright, smooth 40 coating of tin on cold-rolled steel comprising simultaneously electroplating said steel with tin and nickel in such manner that the resulting electrodeposit consists preponderantly of tin and contains about 0.5% to 2% by weight of nickel and 45 thereafter heating the electroplated steel under substantially non-oxidizing conditions to a temperature of about 230° to 260° C.

11. An article of manufacture comprising cold 50 rolled steel coated with a fused metal coating 55 which is preponderantly of tin and which contains another metal selected from the group consisting of copper, nickel, silver and cobalt, said coating containing not less than about 0.4% by weight of said other metal if said other metal is nickel or cobalt and not less than about 1.4% by weight of said other metal if said other metal is copper or silver.

12. An article of manufacture comprising cold-rolled steel coated with a smooth, bright, fused 60 electrodeposit which is preponderantly of tin and which contains 1.4 to 15% by weight of copper.

13. An article of manufacture comprising a cold-rolled steel surface coated with a smooth, bright, fused electrodeposit which is preponderantly of tin and which contains 0.4 to 2% by weight of nickel.

FLOYD FRANCIS OPLINGER.